# EUROPEAN PATENT SPECIFICATION

(11) **EP 0 342 871 B1**
(45) Date of publication and mention of the grant of the patent: **14.04.1993**
(21) Application number: 89304814.0
(22) Date of filing: 11.05.1989
(51) Int. Cl.: C10M 161/00

(54) **Lubricating oil additive concentrate composition**
Schmiermittelzusatzkonzentrat
Composition concentrée d'additifs pour huile lubrifiante

(30) Priority: 14.05.1988 GB 8811473
(43) Date of publication of application: 23.11.1989
(73) Proprietor: BP CHEMICALS (ADDITIVES) LIMITED, London SW1W 0SU (GB)
(72) Inventor: Garner, Anthony, Hedon Hull, HU12 8DS (US); Kikabhai, Thakor, Hedon Hull, HU12 8DS (US)
(74) Representative: Richardson, Derek

(56) References cited:
- EP-A- 0 208 560
- EP-A- 0 264 247
- EP-A- 0 307 132
- GB-A- 1 365 311
- GB-A- 2 048 935
- US-A- 3 697 428

## Description

The present invention relates generally to lubricating oil additive concentrate compositions and their use in finished lubricating oil compositions. In particular the present invention relates to lubricating oil additive concentrate compositions having both dispersancy/detergency properties and viscosity improving properties and their use in finished lubricating oil compositions.

It is known that polyisobutylenes of medium to high molecular weight, for example weight average molecular weights above about 10,000, typically greater than 40,000, act as viscosity index improvers in lubricating oil compositions. Such viscosity index improvers, for example polyisobutylenes having average molecular weights of 60,000 to 80,000 or more, exhibit virtually no dispersant or detergent properties. That is, they are monofunctional additives imparting to the lubricant only the desired viscosity index improving properties. To obtain dispersant or detergent properties, such hydrocarbon viscosity index improvers are used in combination with one or more dispersant or detergent additives.

It is also known that polyisobutylenes can be converted into detergent/dispersant additives for lubricating oil compositions. Thus, for example, the patent literature discloses the preparation of high molecular weight carboxylic acid acylating agents by reacting a polyisobutylene usually containing at least about 50 aliphatic carbon atoms with an unsaturated carboxylic acid or a derivative thereof, for example acrylic acid, fumaric acid and maleic anhydride, see for example US-A-3,024,237; US-A-3,087,936; US-A-3,172,892; US-A-3,215,707; US-A-3,219,666; US-A-3,231,587; US-A-3,245,910; US-A-3,272,746; GB-A-1,085,903; GB-A-1,162,436, GB-A-1,440,219 and many more, the foregoing only being representative of the many patent publications in this area. These same patents also establish that various derivatives, for example the succinimide derivatives, of these high molecular weight carboxylic acid acylating agents are known to be useful as additives in fuel and lubricant compositions, especially as dispersant/detergent additives, which function to promote engine cleanliness, neutralise acidic by-products of combustion, and the like. Some of the compositions disclosed in the above patents have been used in substantial amounts as commercial lubricant additives. The aforesaid derivatives of high molecular weight acylating agents exhibit substantially no viscosity index improver properties. That is they too are essentially monofunctional additives imparting to the lubricant only the desired dispersancy and detergency properties. To obtain viscosity index improver properties such dispersant/detergent additives are generally used in combination with a viscosity index improver additive.

More recently, there has been a move towards multifunctional additives, that is a single additive which exhibits both viscosity index improver and dispersant/detergent properties. In general, two approaches have been used to prepare multifunctional lubricant additives which exhibit both (a) fluidity modifying properties, especially viscosity index improver properties, and (b) dispersant and/or detergent properties. One approach involves "suspending" from or "incorporating" into the hydrocarbon backbone of a high molecular weight polymer certain polar groups (usually carboxylic acid derivatives such as amides and esters). The high molecular weight material so-produced continues to exhibit viscosity index improver properties attributable to its high molecular weight hydrocarbon backbone and dispersant/detergent properties attributable to the polar groups. This approach is illustrated by US-A-3,702,300 and US-A-3,933,761. The second general approach for preparing multifunctional lubricant additives involves modifying a dispersant/detergent additive so as to incorporate into the dispersant/detergent additive fluidity modifying properties, especially viscosity index improver properties. This approach is illustrated by US-A-3,219,666. This patent is mainly concerned with acylated nitrogen derivatives of high molecular weight succinic acid acylating agents, which derivatives function as dispersant additives in lubricant compositions. The acylating agents from which the dispersants are prepared are substituted succinic acylating agents preferably having a substituent derived from a polyisobutylene having a molecular weight of about 750-5000. However, the patent teaches that, if viscosity index improving properties are desired in addition to the dispersant properties, the substituent should be derived from higher molecular weight polyisobutylene polymers, having molecular weights from about 10,000 to about 100,000 or higher. A third approach for preparing lubricant additives having both detergency and viscosity index-improving properties is described in US-A-3,630,902. This approach involves reacting a high molecular weight succinimide with a polymerisable acid to form a polymerisable acyl derivative of the succinimide. The polymerisable derivative is then polymerised to produce the desired multifunctional lubricant additive.

A further approach to the production of a multifunctional lubricating oil additive is described in GB-A-1,565,627. This patent provides a lubricating composition comprising a major amount of oil of lubricating viscosity and a minor amount of one or more carboxylic derivatives produced by reacting at least one substituted succinic acylating agent with a reactant selected from (a) an amine having within its structure at least one H-N〈 group, (b) an alcohol, (c) a reactive metal or reactive metal compound, and (d) a combination of two or more of any of (a) to (c), the components of (d) being reacted with said one or more substituted succinic acylating agents simultaneously or sequentially in any order, wherein said substituted succinic acylating agent(s) consist of substituent groups and succinic groups wherein the substituent groups are derived from polyalkene, preferably polyisobutylene, said polyalkene having an Mn value of 1300 to 5000 and a Mw/Mn value of 1.5 to 4, said acylating agent(s) having within their structure an average of at least 1.3 succinic groups for each equivalent weight of substituent groups.

The only method described for producing the substituted acylating agents of GB-A-1,565,627 is via a chlorination route, which can result in chlorine residues in the final product. The presence of chlorine is undesirable because it can have deleterious effects in engines in which the finished lubricating oil is employed.

Lubricating oil additive packages are normally manufactured by an additive producer and sold on for blending into finished lubricating oils. The additive package generally consists of a mixture of dispersants, detergents, extreme pressure/anti-wear agents, rust inhibitors and other additives for special applications. This package can be used at levels of between 1% and 25% in oil in the automotive field, and up to 40% in the marine field. In addition in the automotive field a viscosity index improver is added if multigrade performance is required. The addition of viscosity index improvers (high molecular weight) to the normal package results in precipitation of the viscosity index improver (VII) rubber and/or the other components in the package. This is due to lack of solvent base oil in the additive carrier oil. This precipitation can be instantaneous or it can occur over a period of 1 day to 180 days or longer. However long the period over which precipitation occurs, it is clearly undesirable. The VII can be a hydrocarbon VII of the ethylene/propylene (EP) copolymer, ethylene/propylene/diene (EPDM), polyisobutene (PIB), polystyrene, hydrogenated polyisoprene, hydrogenated polystyrene/butadiene types etc, or it can be a dispersant polymer such as a polymethacrylate, a dispersant EP, a dispersant EPDM or a dispersant PIB.

In the present invention we have achieved by advantageous blending of PIBs a dispersant which not only has all the dispersant properties of a normal dispersant but also has a small VII contribution to the finished oil and most importantly it has complete compatability with all of the other additives in a typical additive package at conventionally used levels. The blending of the PIBs can take place either before maleanisation and imidation and/or after maleanisation and imidation or at any time during the respective processes.

The use of mixtures of derivatives of polyisobutene-substituted succinic acylating agents in which the polyisobutene substituents have different molecular weights as additives is known in relation to fuels. Thus, GB-A-1,398,067 discloses a detergent additive for a hydrocarbon distillate fuel comprising a mixture of a high molecular weight hydrocarbyl amine and a low molecular weight hydrocarbyl amine, the high molecular weight hydrocarbyl amine containing at least one hydrocarbyl group having an average molecular weight in the range of from 1900 to 5000 and the low molecular weight hydrocarbyl amine containing at least one hydrocarbyl group having an average molecular weight in the range from 300 to 600, the weight ratio of low molecular weight hydrocarbyl amine to high molecular weight hydrocarbyl amine being in the range 0.5:5:1. Although primarily directed to hydrocarbon distillate fuel usage, it is mentioned in the specification that the mixture of high and low molecular weight hydrocarbyl amines may also be used as dispersants and detergents in lubricating oils. Such a mixture, first of all in relation to the low molecular weight hydrocarbyl amine has a hydrocarbyl group of a lower molecular weight than the lowest molecular weight useful in the composition of the present invention, and secondly lacks an essential property of the compositions of the present invention in that there is no component present of a molecular weight sufficiently high to impart adequate viscosity index improver properties to the composition.

According to the present invention there is provided a concentrate composition for use as a multifunctional additive in finished lubricating oils which composition as a first component comprises an oil of lubricating viscosity, as a second component a derivative of a polyisobutylene-subsituted succinic acylating agent wherein the polyisobutylene substituent has a number average molecular weight in the range from about 700 to about 1475, as a third component a derivative of a polyisobutylene-substituted succinic acylating agent wherein the polyisobutylene substituent has a number average molecular weight in the range from about 1500 to about 5000 and as a fourth component a polyisobutylene having a number average molecular weight in the range from about 40,000 to about 400,000, the derivatives being formed by reacting the acylating agents either individually or in combination with either (a) an amine having within its structure at least one H-N group, (b) an alcohol, (c) a reactive metal or reactive metal compound, or (d) a mixture of at least two of (a) to (c), the components of (d) being reacted with the acylating agent(s) either simultaneously or sequentially in any order, the polyisobutylene substituent of the second component forming from 30 to 94.8% by weight of the total polyisobutylene present in the composition, the polyisobutylene substituent of the third component forming from 5 to 69.8% by weight of the total polyisobutylene present in the composition and the polyisobutylene forming the fourth component forming from 0.2 to 5% by weight of the total polyisobutylene present in the composition.

The concentrate composition may simply be formed by mixing the individual components in the lubricating oil. However, it is preferred to produce a mixture of the second and third components by the steps of:-
(I) reacting a mixture of a polyisobutylene having a number average molecular weight in the range from about 700 to about 1475 and a polyisobutylene having a number average molecular weight in the range from about 1500 to about 5000 with an unsaturated carboxylic acid or anhydride thereof to produce a mixture of polyisobutylene-substituted succinic acylating agents, and
(II) reacting the mixture obtained in step (I) with either (a) an amine having within its structure at least one H-N group, (b) an alcohol, (c) a reactive metal or reactive metal compound, or (d) a mixture of at least two of (a) to (c), the components of (d) being reacted with the acylating agent(s) either simultaneously or sequentially in any order.

The mixture obtained in steps (I) and (II) may thereafter be dissolved in the lubricating oil of the first component containing the polyisobutylene fourth component or may be mixed with the fourth component and the mixture dissolved in the lubricating oil.

In a modification of the aforesaid method the polyisobutylene having a number average molecular weight in the range from about 40,000 to 400,000 may be incorporated into the composition by mixing with the polyisobutylenes of number average molecular weight in the range 700 to 1475 and 1500 to 5000 respectively, reacting the mixture so-obtained in step (I) with the carboxylic acid to produce a mixture of polyisobutylene-substituted succinic acylating agents and unreacted polyisobutylene having a number average molecular weight in the range about 40,000 to about 400,000 and thereafter reacting with (a) to (d) in step (II). The amount of derivatised polyisobutylene of number average molecular weight in the range from about 40,000 to about 400,000 in the final composition resulting from the modified preparative method will be relatively small because of the relatively small number of reactive sites present in such high molecular weight materials.

The present invention also provides a finished lubricating oil composition comprising a major proportion of an oil of lubricating viscosity and a minor proportion of the concentrate composition as hereinbefore described.

Suitably the amount of the concentrate composition in the finished lubricating oil may be in the range from 0.01 to 10% by weight.

Polyisobutylenes having number average molecular weights in the range from 700 to 1475, 1500 to 5000 and 40,000 to 400,000 are available commercially, for example from BP Chemicals Limited (Hyvis [RTM]), and may be used without further processing.

The succinic acylating moiety of the polyisobutylene-substituted succinic acylating agent may suitably have the formula:
wherein X and X¹ are the same or different provided that at least one of X and X¹ is such that the substituted succinic acylating agents can function as carboxylic acylating agents. That is, at least one of X and X¹ must be such that the substituted acylating agent can esterify alcohols, form amides or amine salts with ammonia or amines, form metal salts with reactive metals or basic metal compounds, and otherwise function as a conventional carboxylic acid acylating agent.

Thus X and/or X¹ may be -OH, -0-hydrocarbyl, -0⁻M⁺ where M⁺ represents one equivalent of a metal, ammonium or amine cation, -NH₂, -Cl, -Br, and together, X and X¹ can be -0- so as to form the anhydride. The specific identity of any X or X¹ group which is not one of the foregoing is not critical so long as its presence does not prevent the remaining group from entering into acylation reactions. Preferably, however, X and X¹ are such that both carboxyl functions of the succinic group can enter into acylation reactions.

One of the unsatisfied valencies in the grouping
of the formula (I) forms a carbon to carbon bond with a carbon in the substituent group. While other such unsatisfied valence may be satisfied by a similar bond with the same or different substituent group, all but the one aforesaid valence is usually satisfied by hydrogen.

The succinic groups will generally correspond to the formula:-
wherein R and R¹ are each independently either -OH, -Cl, 0-lower alkyl or taken together are -0-. In the latter case the succinic group is a succinic anhydride group. Preferably, the succinic group will corresponds to

The polyisobutene-substituted succinic acylating agents may be prepared in known manner by reacting a polyisobutylene or mixture as aforesaid with one or more of maleic acid, maleic anhydride, fumaric acid or fumaric anhydride, preferably either maleic acid or maleic anhydride. It is preferred to employ the thermal route in preference to the chlorination route as described in GB-A-1565627 in order to avoid contamination of the product with chlorine.

The polyisobutylene-substituted succinic acylating agent(s) is then reacted with (a) to (d) in known manner. As regards the amine (a) this may be either a monoamine or a polyamine. Preferably the amine contains at least one primary amino group and more preferably the amine is a polyamine, most preferably a polyamine containing at least two H - N groups, either or both of which are primary or secondary. Suitable amines and polyamines are described in, for example, US-A-3,087,936 and GB-A-1,565,627, the relevant content of which is incorporated by reference herein. Preferred amines (a) include diethylene triamine, triethylene tetramine and tetraethylene pentamine.

As regards the alcohol (b), this may be either a monohydric or a polyhydric alcohol, polyhydric alcohols being preferred. Suitable alcohols are described in GB-A-1,565,627, the relevant content of which is incorporated herein by reference.

Reactive metals and reactive metal compounds (c) are those which are known to form salts and complexes when reacted with carboxylic acid and carboxylic acid acylating agents. Further details of suitable compounds are disclosed in GB-A-1 ,565,627 the relevant parts of which are incorporated by reference herein.

The oil of lubricating viscosity present in both the concentrate composition and the finished lubricating oil composition may be the same or different. The oil may be a natural oil or a synthetic oil or a mixture of oils. Suitable oils are those described in GB-A-1,565,627, the disclosure of which is incorporated by reference herein.

The finished lubricating oil may contain additional additives conventionally employed in lubricating oils. These may be added directly to the finished lubricating oil composition or may be added in the concentrate composition.

The concentrate composition of the present invention imparts to lubricating oils an increase in their high temperature viscosity characteristics whilst retaining or improving their low temperature viscosity characteristics and providing dispersancy/detergency properties. We have attempted to express the viscosity characteristics by the following relationship:-
- Numerical gradient: = 100 x (HTV_{compound oil} - HTVₒᵢₗ)/(LTVₒᵢₗ - HTVₒᵢₗ)
- where HTV_{compound oil}: = High temperature viscosity of the compounded oil.
- HTVₒᵢₗ: = High temperature viscosity of the lubricating oil.
- LTVₒᵢₗ: = Low temperature viscosity of the lubricating oil.

Whereas this gradient for the succinimide derivative of either of the second and third components or their combination does not exceed about 11, the gradient for the succinimide derivatives of the second and third components in admixture with the fourth component is about 18.

The invention will now be further illustrated by reference to the following Examples and Comparison Tests.

In the following Examples and Comparison Tests the following commercially available polyisobutenes were employed:-

### Test

Different materials were blended into oil with the aim of improving viscometric performance compared to commercially available materials. The acceptance criterion for improved viscometrics were (at 5% in 150 SN lubricating oil):-
V₁₀₀ greater than or equal to 6.9 mm²/s (cSt)
and
V₋₂₀ less than or equal to 40 mm²/s

### Comparison Tests 1 - 3

The viscometric characteristics of three commercially available dispersants were determined at 10% in 150 SN lubricating oil. The results are given in Table 1.

All the commercially available dispersants tested were viscometrically acceptable.

### Comparison Tests 4 - 9

The viscometric characteristics of six commercially available polyisobutenes [(A) to (F)] were determined at 5% in 150 SN lubricating oil. The results are given in Table 2.

None of the commercially available polyisobutenes tested met the viscometrics acceptance criterion.

### Comparison Tests 10 to 17

The viscometric characteristics of eight blends of two commercially available polyisobutenes were determined at 5% in 150 SN lubricating oil. The results are given in Table 3.

Although some of the polyisobutene two-component blends met the viscometric acceptance criterion, the criterion was not consistently met.

### Examples 1 to 5

The viscometric characteristics of five three-component polyisobutene blends were determined at 5% in 150 SN lubricating oil. The results are given in Table 4.

The three-component blends consistently meet the viscometric acceptance criterion.

## Claims

1. A concentrate composition for use as a multifunctional additive in finished lubricating oils which composition as a first component comprises an oil of lubricating viscosity, as a second component a derivative of a polyisobutylene-substituted succinic acylating agent wherein the polyisobutylene substituent has a number average molecular weight in the range from about 700 to about 1475, as a third component a derivative of a polyisobutylene-substituted succinic acylating agent wherein the polyisobutylene-substituent has a number average molecular weight in the range from about 1500 to about 5000 and as a fourth component a polyisobutylene having a number average molecular weight in the range from about 40,000 to about 400,000, the derivatives being formed by reacting the acylating agents either individually or in combination with either (a) an amine having within its structure at least one H-N〈 group, (b) an alcohol, (c) a reactive metal or reactive metal compound, or (d) a mixture of at least two of (a) to (c), the components of (d) being reacted with the acylating agent(s) either simultaneously or sequentially in any order, the polyisobutylene substituent of the second component forming from 30 to 94.8% by weight of the total polyisobutylene present in the composition, the polyisobutylene substituent of the third component forming from 5 to 69.8% by weight of the total polyisobutylene present in the composition and the polyisobutylene forming the fourth component forming from 0.2 to 5% by weight of the total polyisobutylene present in the composition.

2. A concentrate composition according to claim 1 wherein a mixture of the second and third components is produced by the steps of:-
(I) reacting a mixture of a polyisobutylene having a number average molecular weight in the range from about 700 to about 1475 and a polyisobutylene having a number average molecular weight in the range from about 1500 to about 5000 with an unsaturated carboxylic acid or anhydride thereof to produce a mixture of polyisobutylene-substituted succinic acylating agents, and
(II) reacting the mixture obtained in step (I) with either (a) an amine having within its structure at least one H-N group, (b) an alcohol, (c) a reactive metal or reactive metal compound, or (d) a mixture of at least two of (a) to (c), the components of (d) being reacted with the acylating agent(s) either simultaneously or sequentially in any order.

3. A concentrate composition according to claim 2 wherein the mixture obtained in steps (I) and (II) is dissolved in the oil of lubricating viscosity (the first component) containing the polyisobutylene having a number average molecular weight in the range from about 40,000 to about 400,000 (the fourth component).

4. A concentrate composition according to claim 2 wherein the mixture obtained in steps (I) and (II) is mixed with the polyisobutylene having a number average molecular weight in the range from about 40,000 to about 400,000 (the fourth component) and the mixture so-obtained dissolved in the oil of lubricating viscosity (the first component).

5. A concentrate composition according to claim 2 wherein the polyisobutylene having a number average molecular weight in the range from about 40,000 to 400,000 (the fourth component) is incorporated into the composition by mixing with the polyisobutylenes of number average molecular weight in the range 700 to 1475 and 1500 to 5000 respectively, reacting the mixture so-obtained in step (I) with the carboxylic acid to produce a mixture of polyisobutylene-substituted succinic acylating agents and unreacted polyisobutylene having a number average molecular weight in the range about 40,000 to about 400,000 and thereafter reacting with either (a) to (d) in step (II).

6. A concentrate composition according to any one of the preceding claims wherein the polyisobutylene-substituted succinic acylating agents are prepared by reacting a polyisobutylene or mixture thereof with one or more of maleic acid or maleic anhydride.

7. A concentrate composition according to claim 6 wherein reaction is effected by the thermal route.

8. A concentrate composition according to any one of the preceding claims wherein the derivative is formed by reacting the acylating agent with an amine which is either diethylene triamine, triethylene tetramine or tetraethylene pentamine.

9. A finished lubricating oil composition comprising a major proportion of an oil of lubricating viscosity and a minor proportion of the concentrate composition of claims 1 to 8.

10. A finished lubricating oil composition according to claim 9 wherein the amount of the concentrate composition in the finished composition is in the range from 0.01 to 10% by weight.

## Patentansprüche

1. Konzentrat-Zusammensetzung zur Verwendung als ein multifunktionelles Additiv in fertiggestellten Schmierölen, die als eine erste Komponente ein Öl von Schmierviskosität, als eine zweite Komponente ein Derivat eines Polyisobutylen-substituierten Bernsteinsäureacylierungsmittels, worin der Polyisobutylen-Substituent ein Zahlenmittel-Molekulargewicht im Bereich von etwa 700 bis etwa 1475 aufweist, als eine dritte Komponente ein Derivat eines Polyisobutylen-substituierten Bernsteinsäureacylierungsmittels, worin der Polyisobutylen-Substituent ein Zahlenmittel-Molekulargewicht im Bereich von etwa 1500 bis etwa 5000 aufweist, und als eine vierte Komponente ein Polyisobutylen mit einem Zahlenmittel-Molekulargewicht im Bereich von etwa 40 000 bis etwa 400 000, enthält, wobei die Derivate durch Umsetzen des acylierenden Mittels entweder einzeln oder in Kombination mit entweder (a) einem Amin, das in seiner Struktur zumindest eine H-N< Gruppe enthält, (b) einem Alkohol, (c) einem reaktiven Metall oder einer reaktiven Metallverbindung, oder (d) einer Mischung von zumindest zwei der Komponenten von (a) bis (c), gebildet werden, wobei die Komponenten von (d) mit dem bzw. den acylierenden Mitteln entweder gleichzeitig oder nacheinander in beliebiger Reihenfolge umgesetzt werden, der Polyisobutylen-Substituent der zweiten Komponente von 30 bis 94,8 Gewichtsprozent des gesamten in der Zusammensetzung vorhandenen Polyisobutylens ausmacht, der Polyisobutylen-Substituent der dritten Komponente von 5 bis 69,8 Gewichtsprozent des gesamten in der Zusammensetzung vorhandenen Polyisobutylens ausmacht und das die vierte Komponente bildende Polyisobutylen von 0,2 bis 5 Gewichtsprozent des gesamten in der Zusammensetzung vorhandenen Polyisobutylens ausmacht.

2. Konzentrat-Zusammensetzung nach Anspruch 1, **dadurch gekennzeichnet,** daß man eine Mischung der zweiten und dritten Komponenten durch die nachfolgenden Stufen herstellt:
(I) Umsetzen einer Mischung eines Polyisobutylens mit einem Zahlenmittel-Molekulargewicht im Bereich von etwa 700 bis etwa 1475 und einem Polyisobutylen mit einem Zahlenmittel-Molekulargewicht im Bereich von etwa 1500 bis etwa 5000 mit einer ungesättigten Carbonsäure oder einem Anhydrid derselben zur Bildung einer Mischung von Polyisobutylensubstituierten Bernsteinsäureacylierungsmitteln, und
(II) Umsetzen der in Stufe (I) erhaltenen Mischung mit entweder (a) einem Amin, das innerhalb seiner Struktur zumindest eine H-N< Gruppe aufweist, (b) einem Alkohol, (c) einem reaktiven Metall oder einer reaktiven Metallverbindung, oder (d) einer Mischung von zumindest zwei der unter (a) bis (c) genannten Verbindungen, wobei die Komponenten von (d) mit dem oder den acylierenden Mitteln entweder gleichzeitig oder nacheinander in beliebiger Reihenfolge umgesetzt werden.

3. Konzentrat-Zusammensetzung nach Anspruch 2, **dadurch gekennzeichnet,** daß die in den Stufen (I) und (II) erhaltene Mischung in dem Öl von Schmierviskosität (der ersten Komponente), enthaltend das Polyisobutylen mit einem Zahlenmittel-Molekulargewicht im Bereich von etwa 40 000 bis etwa 400 000 (die vierte Komponente), aufgelöst wird.

4. Konzentrat-Zusammensetzung nach Anspruch 2, **dadurch gekennzeichnet,** daß die in den Stufen (I) und (II) erhaltene Mischung mit dem Polyisobutylen mit einem Zahlenmittel-Molekulargewicht im Bereich von etwa 40 000 bis etwa 400 000 (der vierten Komponente) gemischt und die so erhaltene Mischung in dem Öl von Schmierviskosität (der ersten Komponente) aufgelöst wird.

5. Konzentrat-Zusammensetzung nach Anspruch 2, **dadurch gekennzeichnet,** daß das Polyisobutylen mit einem Zahlenmittel-Molekulargewicht im Bereich von etwa 40 000 bis 400 000 (die vierte Komponente) in die Zusammensetzung durch Mischen mit den Polyisobutylenen mit Zahlenmittel-Molekulargewicht im Bereich von 700 bis 1475 bzw. 1500 bis 5000 inkorporiert wird, Umsetzen der so erhaltenen Mischung in Stufe (I) mit der Carbonsäure zur Herstellung einer Mischung von Polyisobutylen-substituierten Bernsteinsäureacylierungsmitteln und nichtumgesetztem Polyisobutylen mit einem Zahlenmittel-Molekulargewicht im Bereich von etwa 40 000 bis etwa 400 000, und anschließendes Umsetzen mit entweder (a) bis (d) in Stufe (II).

6. Konzentrat-Zusammensetzung nach irgendeinem der vorhergehenden Ansprüche, **dadurch gekennzeichnet**, daß die Polyisobutylen-substituierten Bernsteinsäureacylierungsmittel durch Umsetzen eines Polyisobutylens oder einer Mischung daraus mit einer oder mehr Verbindungen von Maleinsäure oder Maleinsäureanhydrid hergestellt werden.

7. Konzentrat-Zusammensetzung nach Anspruch 6, **dadurch gekennzeichnet**, daß die Reaktion auf dem thermischen Weg durchgeführt wird.

8. Konzentrat-Zusammensetzung nach irgendeinem der vorhergehenden Ansprüche,**dadurch gekennzeichnet,** daß das Derivat durch Umsetzen des acylierenden Mittels mit einem Amin, welches entweder Diethylentriamin, Triethylentetramin oder Tetraethylenpentamin ist, gebildet wird.

9. Fertiggestellte Schmieröl-Zusammensetzung, **dadurch gekennzeichnet**, daß sie eine Hauptmenge eines Öls von Schmierviskosität und eine kleinere Menge der Konzentrat-Zusammensetzung der Ansprüche 1 bis 8 enthält.

10. Fertiggestellte Schmieröl-Zusammensetzung nach Anspruch 9, **dadurch gekennzeichnet,** daß die Menge der Konzentrat-Zusammensetzung in der fertiggestellten Zusammensetzung im Bereich von 0,01 bis 10 Gewichtsprozent liegt.

## Revendications

1. Composition concentrée destinée à être utilisée comme additif multifonctionnel dans des huiles lubrifiantes finales, composition succinique substitué par un polyisobutylène dans lequel le substilubrifiante, comme second composant, un dérivé d'un agent d'acylation succinique substitué au polyisobutylène dans lequel le substituant polyisobutylène a un poids moléculaire moyen en nombre de l'ordre d'environ 700 à environ 1475, comme troisième composant, un dérivé d'un agent d'acylation succinique substitué au polyisobutylène dans lequel le substituant polyisobutylène a un poids moléculaire moyen en nombre de l'ordre d'environ 1500 à environ 5000 et, comme quatrième composant, un polyisobutylène ayant un poids moléculaire moyen en nombre de l'ordre d'environ 40 000 à environ 400 000, les dérivés étant formés par réaction des agents d'acylation soit individuellement, soit en combinaison, avec soit (a) une amine ayant dans sa structure au moins un groupe H-N〈 , (b) un alcool, (c) un métal réactif ou un composé métallique réactif, soit (d) un mélange d'au moins deux des composés de (a) à (c), les composants de (d) étant obtenus par réaction soit simultanément, soit en séquence, dans n'importe quel ordre, avec l'agent (les agents) d'acylation, le substituant polyisobutylène du second composant constituant de 30 à 94,8% en poids du polyisobutylène total présent dans la composition, le substituant polyisobutylène du troisième composant constituant de 5 à 69,8% en poids du polyisobutylène total présent dans la composition et le polyisobutylène formant le quatrième composant constituant de 0,2 à 5% en poids du polyisobutylène total présent dans la composition.

2. Composition concentrée suivant la revendication 1, dans laquelle un mélange des second et troisième composants est produit par les étapes consistant à:
(I) faire réagir un mélange d'un polyisobutylène ayant un poids moléculaire moyen en nombre de l'ordre d'environ 700 à environ 1475 et un polyisobutylène ayant un poids moléculaire moyen en nombre de l'ordre d'environ 1500 à environ 5000 avec un acide carboxylique non-saturé ou un anhydride de celui-ci pour produire un mélange d'agents d'acylation succiniques substitués par le polyisobutylène et
(II) faire réagir le mélange obtenu à l'étape (I) avec soit (a) une amine ayant dans sa structure au moins un groupe H-N , (b) un alcool, (c) un métal réactif ou un composé métallique réactif, soit (d) un mélange d'au moins deux des composés de (a) à (c), les composants de (d) étant obtenus par réaction soit simultanément, soit en silence, dans n'importe quel ordre, avec l'agent (les agents) d'acylation.

3. Composition concentrée suivant la revendication 2, dans laquelle le mélange obtenu aux étapes (I) et (II) est dissous dans l'huile à viscosité lubrifiante (le premier composant) contenant le polyisobutylène ayant un poids moléculaire moyen en nombre de l'ordre d'environ 40 000 à environ 400 000 (le quatrième composant).

4. Composition concentrée suivant la revendication 2, dans laquelle le mélange obtenu aux étapes (I) et (II) est mélangé au polyisobutylène ayant un poids moléculaire moyen en nombre de l'ordre d'environ 40 000 à environ 400 000 (le quatrième composant) et le mélange ainsi obtenu est dissous dans l'huile à viscosité lubrifiante (le premier composant).

5. Composition concentrée suivant la revendication 2, dans laquelle le polyisobutylène ayant un poids moléculaire moyen en nombre de l'ordre d'environ 40 000 à environ 400 000 (le quatrième composant) est incorporé à la composition par mélange avec les polyisobutylènes à poids moléculaire moyen en nombre de l'ordre de, respectivement, 700 à 1475 et 1500 à 5000, réaction du mélange ainsi obtenu à l'étape (I) avec l'acide carboxylique pour produire un mélange d'agents d'acylation succiniques substitués par le polyisobutylène et du polyisobutylène n'ayant pas réagit ayant un poids moléculaire moyen en nombre de l'ordre d'environ 40 000 à environ 400 000 et, ensuite, réaction avec l'un ou l'autre des composés de (a) à (d) à l'étape (II).

6. Composition concentrée suivant l'une ou l'autre des revendications précédentes, dans laquelle les agents d'acylation succiniques substitués au polyisobutylène sont préparés par réaction d'un polyisobutylène ou mélange de celui-ci avec un ou plusieurs acides parmi l'acide maléique ou l'anhydride maléique.

7. Composition concentrée suivant la revendication 6, dans laquelle la réaction se fait par la voie thermique.

8. Composition concentrée suivant l'une ou l'autre des revendications précédentes, dans laquelle le dérivé est formé par réaction de l'agent d'acylation avec une amine qui est soit la triamine de diéthylène, soit la tétramine de triéthylène. soit la pentamine de tétraéthylène.

9. Composition d'huile lubrifiante. finale comprenant une grande proportion d'une huile à viscosité lubrifiante et une petite proportion de la composition concentrée suivant les revendications 1 à 8.

10. Composition d'huile lubrifiante finale suivant la revendication 9, dans laquelle la quantité de la composition concentrée dans la composition finale est de l'ordre de 0,01 à 10% en poids.
